

A. THOMA.  
Refining Steel.

No. 70,048.

Patented Oct. 22, 1867.



Witnesses.

Theo Fischer  
Wm. Treurn

Inventor.  
A. Thoma  
Per *John C. Ottomys*

# United States Patent Office.

ALOIS THOMA, OF NEW YORK, N. Y., ASSIGNOR TO HIMSELF, S. BROMBERG,  
AND ARTEMUS W. WILDER, OF SAME PLACE.

*Letters Patent No. 70,048 dated October 22, 1867.*

## IMPROVED FURNACE FOR MELTING AND PURIFYING STEEL.

The Schedule referred to in these Letters Patent and making part of the same.

TO ALL WHOM IT MAY CONCERN:

Be it known that I, ALOIS THOMA, of the city, county, and State of New York, have invented a new and improved Furnace for Smelting Steel; and I do hereby declare that the following is a full, clear, and exact description thereof, which will enable others skilled in the art to make and use the same, reference being had to the accompanying drawings, forming a part of this specification, in which—

Figure 1 represents a horizontal sectional view of my improved smelting-furnace, the plane of section being indicated by the line *x x*, fig. 2.

Figure 2 is a longitudinal central sectional elevation of the same.

Figure 3 is an end view, partly in section, of the same.

Similar letters of reference indicate corresponding parts.

This invention relates to a new furnace for smelting steel, and for producing cast steel of the best quality from steel of ordinary or inferior kind. To do this, I melt the steel in an open pan or vessel, which is fitted in a suitable furnace. Heretofore steel had to be molten in crucibles, which are not only very expensive, but which also require a very large amount of heat to melt the material in their inside. By doing away with the use of the crucibles, and by melting the steel in an open pan, I reduce the expense of the steel-smelting process to a considerable degree, as the pan is not only much cheaper, and can be used frequently, but as, also, considerable fuel is saved, the steel being molten much quicker than in the crucibles. Furthermore, the arrangement of my furnace does not confine me to the use of any certain kind of fuel, and the expense of smelting may thus be still more reduced by using a cheaper kind of fuel.

A represents a furnace, made of fire-brick or other suitable material, and consisting of three main divisions: the fireplace B, the melting-oven C, and the air-heating chamber D. The chambers B and C are connected by a channel, *a*, and the chambers C and D by a channel, *b*, as shown in fig. 2. In the fireplace B are arranged a suitable grate, *c*, and a channel, *e*, above it, to put in the fuel. A door, *d*, in the end of the furnace, can be used for cleaning the fireplace. *f* is a pipe for conducting the requisite amount of draught to the fire; *g* is the ash-pit, and *h* a door to the same. The channel *a*, through which the flame passes to the oven C, inclines towards the oven, as shown in fig. 2. Above the channel *a* is arranged, in the furnace, a pipe or reservoir, *i*, from which an opening, *j*, extends to the channel *a*, connecting the same with the reservoir *i*, as is clearly shown in fig. 2. The opening *j* is arranged obliquely, and wider at its lower end, so that a blast of air blown through it will throw the flame upon the surface of the channel *a*, and detain it there for a short time, and will also force the flame over and through the surface of the steel in the oven. As the blast forces the flames down, they are retarded in their progress, and thereby all dust that might arise from the fuel will be retained, and will be prevented from being carried off by the flame. Thereby the flame is purified, which it must be in order to produce pure cast steel. All the gases carried off with the flame will be completely burned by the action of the blast, and a most intense heat will be created in the channel *a*.

The interior of the hearth or oven C can be reached through doors *k* *k'*, arranged in the opposite sides of the same. Through the smaller door *k* the oven is filled and emptied, while through the larger door *k'* the pan *l* is inserted. This pan consists of three, more or less, sections, which, when arranged together, form an open, shallow pan or vessel, *l*, which corresponds in its outer shape to the shape of the oven C.

The hearth is made of good fire-brick or other suitable material. Upon its surface is placed a layer of good quartz-sand, which must be well levelled and firmly stamped. Then the sections of the pan are inserted through the door *k'*, so that they will rest upon the sand-sole *m*. A small space should be left between the rim of the pan and the wall of the oven, which is filled, as well as the crevices between the sections of the pan, with quartz-sand which has been mixed in wet clay. The upper parts of these crevices are filled with a mixture of quartz, lime, and salt. When heat is applied, this latter mixture will melt, and will connect the sections of the pan so as to make a smooth bottom in the pan, while the addition of the quartz makes this cement so brittle that it can be easily broken when the pan is to be removed from the furnace.

The pan *l*, as well as the inner lining of the oven, is best made of good fire-brick clay, pressed, and, when dry, coated on the fire side with concentrated salt solution, and then thoroughly burned.

The flame, after having passed through the oven, escapes through the channel *b* into the air-heating chamber *D*, in which pipe *n* is arranged in zigzag lines. The pipe leads to the reservoir *i*, and carries the blast of air to the fire. The products of combustion, entering the chamber *D*, heat the pipe *n*, and thereby the blast is carried to the fire. These pipes, not being directly in the fire, as usual, cannot leak without it being noticed and easily repaired. The products of combustion are finally carried off through a chimney, *E*.

The steel to be molten is placed in the pan *l*, and covered with a thin layer of fluid dross, which protects it from the direct influence of the flame, so that only the heat of the flame will act upon the steel, but not any gases contained therein.

By the arrangement of the blast-channel *j*, the flame is blown over the surface of the steel, and the heat thus brought against the steel is higher than could ever be produced in any other furnace in which iron or steel is treated, and therefore the smelting process will occupy but comparatively short time. Therefore, also, large quantities of steel can be molten in this furnace.

It is advisable to test the steel during the melting process, so that, if required, its quality can be improved by adding bar iron or hard steel. A hole, *o*, is arranged in the door *k'*, and in the rim of the pan *l*, to discharge the steel when finished. Where crucibles are used, steel cannot be thus treated, improved, or tested during the melting process.

By the Bessemer process of producing steel, good steel for cutting-tools is only accidentally produced, the general quality being impure, mixed with sulphur and phosphorus. Such impure steel can be converted into perfectly pure cast steel in my furnace.

Having thus described my invention, what I claim as new, and desire to secure by Letters Patent, is—

1. Smelting steel in an open pan, by blowing a purified flame over the surface of the steel in the pan, substantially as herein shown and described.

2. The pan *l*, in which the steel to be smelted is placed, when said pan is made in sections, so that it can be easily inserted and removed through the narrow doors of the furnace, substantially as herein shown and described.

3. Connecting the smelting-oven *C* with the air-heating chamber *D*, by means of a chamber, *b*, so that the air pipe *n* is heated in the chamber *D*, and not in the oven *C*, substantially as and for the purpose herein shown and described.

4. So arranging a furnace for smelting steel that the steel can be tested and treated during the smelting process, substantially as herein shown and described.

5. The chambers *C*, *D*, and *E*, when connected by channels *a* and *b*, and when combined with the reservoir *i*, blast-channel *j*, pan *l*, and pipe *n*, all made, arranged, and operating substantially as and for the purpose herein shown and described.

6. Making the blast-channel *j* wider at its lower end, and arranging it obliquely in the furnace, substantially as and for the purpose herein shown and described.

ALOIS THOMA.

Witnesses:

A. V. BRIESEN,

ALEX. F. ROBERTS.